

H. CLARKE & J. A. CAMPBELL.

FUEL.

APPLICATION FILED AUG. 4, 1911. RENEWED JAN. 24, 1916.

1,193,763.

Patented Aug. 8, 1916.



Fig. 1.

Fig. 2.

Witnesses—

Stanley Hood  
Robert Owen Hughes.

Inventors

Herman Clarke  
James A. Campbell  
by  
W. Evans.

Attorney.

# UNITED STATES PATENT OFFICE.

HERMAN CLARKE, OF LONDON, AND JAMES A. CAMPBELL, OF ILFORD, ENGLAND.

## FUEL.

1,193,763.

Specification of Letters Patent. Patented Aug. 8, 1916.

Application filed August 4, 1911, Serial No. 642,357. Renewed January 24, 1916. Serial No. 74,062.

To all whom it may concern:

Be it known that we, HERMAN CLARKE, a citizen of the United States of America, and residing at 3 London Wall Buildings, 5 London, E. C., England, engineer, and JAMES ALEXANDER CAMPBELL, a subject of the King of Great Britain and Ireland, residing at 23 Eton road, Ilford, England, engineer, have invented certain new and useful 10 Improvements Relating to Fuel, of which the following is a specification.

This invention relates to the production of a smokeless fuel by the partial destructive distillation of bituminous or semi-bituminous coal or similar carbonaceous substance, 15 and the invention has for its objects to produce a fuel that will not easily crumble in handling or in carriage, that can be readily discharged from the retort in which it is produced, and in the process of whose production tar is produced uncontaminated with 20 paraffins and capable of profitable distillation yielding a large percentage of hydrocarbons of the benzol series, and tar acids rich in crystallizable orthocresol and pitch 25 of good and tough quality having a low content of free carbon; as well as a considerable quantity of ammoniacal liquor consisting largely of free ammonia; and a gas of high 30 illuminating power and calorific value, containing benzol in considerable quantity.

According to the invention the process of distillation is effected under such conditions as to insure the retention in the residue of a 35 relatively high percentage of volatile matter, and with a view to insure the production of a residue that will not easily crumble in handling or in carriage, the distillation is effected under such conditions as to insure 40 the formation around the charge of an exterior crust of hard coke.

According to the invention, moreover, the distillation is effected within vertical retorts tapered outwardly toward the bottom, and 45 the distillation is arrested when the charge has contracted to such an extent as to be free from the walls of the retort, that is to say, at the stage when, upon the doors being opened, the charge falls out of the retort as 50 an integral mass, without the necessity of employing special means for its withdrawal. By arresting the distillation at this stage a residue is produced having on its exterior a thick crust of hard coke.

55 The invention comprises the process that is hereinafter described.

A retort such as may be employed for carrying out the invention is illustrated in the accompanying drawing, in which—

Figure 1 is a sectional elevation, and Fig. 60 2 a corresponding cross-section taken on the line  $x-y$  of Fig. 1.

In carrying the invention into effect vertical retorts such as  $a$  are preferably employed of oblong section having an internal 65 width of about six inches and of any convenient breadth, each retort  $a$  being advantageously made up in short lengths or sections  $b$  and of fireclay, cast iron or other suitable material, and each length or section 70 of each retort being connected with the other by such means as a spigot and socket or other gas tight connection, by which a continuous vertical retort is formed tapering outwardly 75 toward the bottom door.

The coal or other substance to be distilled and preferably in the form of slack is fed to the retort from the top, where a gas-tight cover  $c$  is mounted. The retort is maintained at about from 1,300° to 1,400° 80 F. for from seven to eight hours, that is to say, until the charge reaches the condition in which it has contracted sufficiently to fall of its own weight and beyond the stage at which the evolution of tar or illuminating 85 gases has ceased. By destructive distillation effected and arrested under these conditions, the residue is surrounded by a crust of hard coke, of from  $\frac{1}{4}$ " to  $\frac{3}{4}$ " in thickness, almost entirely devoid of volatile matter, 90 while the central mass or core of the residue contains sufficient volatile matter (from 6 to 10%) to render it free burning. By such a process of distillation a fuel is produced which, by reason of the crust formed by contact of the walls of the retort with the charge, is adapted to withstand handling 95 and carriage with a very small loss in crumbling, while furthermore a product results which has a high calorific value and is 100 smokeless in combustion.

What we claim as our invention and desire to secure by Letters Patent is:—

1. A new product of manufacture, being a smokeless fuel consisting of a solid body of coke, the greater part of whose mass at the center contains a relatively high proportion of volatile matter and is relatively fragile, the remainder containing a small proportion of volatile matter and forming a relatively 105 hard crust, the whole, however, forming an integral mass.

2. A new product of manufacture, being a smokeless fuel consisting of a solid body of coke, the greater part of whose mass at the center is relatively fragile and has a hard 5 crust integral therewith.

3. A process for the partial destructive distillation of coal or carbonaceous matter, for the production of a fuel, which consists in subjecting the mass in a closed retort to 10 destructive distillation past the stage when illuminating gases have ceased to be evolved and continuing the distillation until the outer portion of the charge in contact with the walls of the retort forms a crust of coke 15 integral with the main mass thereof, and then arresting the distillation substantially as described.

4. A process for the partial destructive distillation of coal or carbonaceous matter 20 and for the production of fuel, consisting in subjecting the mass in a closed vertical retort to destructive distillation past the stage when illuminating gases have ceased to be evolved and continuing the distillation until 25 the charge in the retort shrinks and a hard integral crust is formed around the charge, then arresting the distillation substantially as described.

5. A process for the partial destructive 30 distillation of coal or carbonaceous matter, for the production of a fuel, which consists in subjecting the mass in a closed retort to destructive distillation at a medium temperature past the stage at which illuminating 35 gases have ceased to be evolved and continuing the distillation until the outer portion of the charge in contact with the walls of the retort forms a crust of coke integral with the main mass thereof, and 40 then arresting the distillation substantially as described.

6. A process for the partial destructive distillation of coal or carbonaceous matter,

for the production of a fuel, which consists in subjecting the mass in a closed retort to 45 destructive distillation at about 1300° to 1400° F. past the stage at which illuminating gases have ceased to be evolved and continuing the distillation until the outer portion of the charge in contact with the walls 50 of the retort forms a crust of coke integral with the main mass thereof, and then arresting the distillation substantially as described.

7. A process for the partial destructive 55 distillation of coal or carbonaceous matter and for the production of fuel, consisting in subjecting the mass in a closed vertical retort to a medium temperature past the stage at which illuminating gases have ceased to 60 be evolved and continuing the distillation until the charge in the retort shrinks and a hard integral crust is formed around the charge, then arresting the distillation substantially as described.

8. A process for the partial destructive distillation of coal or carbonaceous matter and for the production of fuel, consisting in subjecting the mass in a closed vertical retort to destructive distillation at about 70 1300° to 1400° F. past the stage at which illuminating gases have ceased to be evolved and continuing the distillation until the charge in the retort shrinks and a hard integral crust is formed around the charge, 75 then arresting the distillation substantially as described.

In testimony whereof we have hereunto signed this specification in the presence of two subscribing witnesses.

HERMAN CLARKE.  
JAS. A. CAMPBELL.

Witnesses:

GEORGE HAM,  
H. W. BLAKE.